

July 8, 1930.

W. M. STERNBERG

1,770,047

TREATMENT OF TEXTILE ELEMENTS OR YARN DERIVED  
FROM RAYON FILAMENTS OR FIBERS

Filed Aug. 27, 1926

Fig. 1.



Fig. 2.



Inventor

W. W. Sternberg

By   
Attorney

## UNITED STATES PATENT OFFICE

WOLDEMAR M. STERNBERG, OF NEW YORK MILLS, NEW YORK, ASSIGNOR TO ROBERT G. CAMPBELL, OF UTICA, NEW YORK

TREATMENT OF TEXTILE ELEMENTS OR YARN DERIVED FROM RAYON FILAMENTS OR FIBERS

Application filed August 27, 1926. Serial No. 131,966.

This invention relates, primarily, to the treatment of textile elements or yarn derived from rayon filaments or fibers; it has especial reference to a method of lusterizing such elements; and it involves a step of stretching the same to a predetermined degree.

It has heretofore been proposed to produce rayon yarn by cutting commercial rayon filaments or fibers to relatively short lengths and then spinning a plurality of these cut sections together to produce a type of textile element or yarn having certain characteristics not possessed by the filaments, themselves, before they are spun together.

The procedure involved in developing this new yarn has a tendency to remove some of the surface luster of the yarn. In other words, the spinning—which involves a twisting of the short-length filaments—seems to have the effect mentioned: That is to say, it is known that when rayon fibers or filaments are twisted together, as by spinning, the luster of the resulting spun yarn is always less than that of the original fibers when they are laid parallel. This loss of luster may be attributed to the fact that on twisting a parallel bunch of fibers or filaments, the latter assume an arrangement in space which is influenced by the inherent rigidity of the component fibers. Each fiber will form a sort of spiral; but these spirals, except only in some instances, furnish no stretches or sections which are parallel to each other. It has been discovered that by partially twisting such spun yarns, the tendency of the fibers thereof is to assume a parallel arrangement for greater lengths, with a resulting improvement of luster. This effect is particularly noticeable when the back-twisting is done with the fibers in the moist state. Such treatment may result in loss of tensile strength of the yarn—due, doubtless, to a decrease in points of contact of the fibers—which causes a break when the yarn is placed under tension, this break being, to a great extent, a slippage of fibers, one past the other.

A similar lusterizing—as effected by back-twisting the yarn—may be produced by stretching it, such action apparently tending to restore the component fibers in parallelism

over increased stretches or sections of the spirals. Artificial fibers and rayon filaments possess great rigidity and resilience. To attain the maximum lusterizing effect, this rigidity must, to a great extent, be overcome, and this can be effectually accomplished by stretching the spun yarn or elements while in a moist state. If such stretched elements be left to dry, then and while under tension, the resulting yarn does have an improved luster and, at the same time, due to improved contact between the fibers, the yarn is very appreciably improved in strength, its internal friction having been increased, and the break becoming dependent less upon the slippage of fibers, and more upon actual rupture of the component filaments.

The improvement of luster and increase in strength are the greater, the higher the tension under which moist yarns are permitted to dry. For that reason, the tensions used have preferably been rather high, approaching as closely as is safe the breaking loads of the wet yarns. Inasmuch as no yarns are entirely uniform throughout their length, the tensions selected have usually been somewhere between one-half ( $\frac{1}{2}$ ) and two-thirds ( $\frac{2}{3}$ ) of the average breaking loads of the wet yarns. It being easier, in practice, to measure a load (tension) applied by the effect it produces upon the stretched (tensioned) yarn, it is my preferred practice to stretch the wet yarn close to ten per cent (10%), and then to permit it to dry while maintaining the stretch unaltered.

In the accompanying drawing, which is more or less diagrammatic, I have illustrated, in two comparative views, the relative position of the fibers or filaments before and after stretching, that is, tensioning. In other words, in Fig. 1, the fibers or filaments are shown in the position they assume during the spinning operation, such filaments being designated by the reference-character 3; while, in Fig. 2, these filaments 3 are shown in the approximate relation they assume as a result of the stretching operation which I have proposed to effect lusterization of the yarn.

In the actual routine of manufacture of yarn, the stretching may be applied at the

different stages of manufacture: For instance, if the yarn is to be bleached or dyed, or will have in any way to pass through a wet state during finishing operations, the obvious place for stretching will be during the subsequent drying. It may be done in skeins (if the finishing operations are made on yarn in the form of skeins; or in continuous strands, by carrying the yarn out of the last wash-water on a system of rollers possessing graded speeds, this operation imparting a stretch to the wet yarn and maintaining it in that condition until the yarn has been passed through a drier and dried.

It may prove advantageous to have the wash-water contain substances in solution or suspension which, when left on the dried yarn, will impart to it some desirable property, such as improved pliability. Thus, a suspension of oil, in proportions of, say, two to three per cent or more, would cause the dry yarn to be lubricated with an amount of oil which would prove adequate in subsequent processes of knitting or weaving.

What I claim is:

1. The method of lusterizing a spun rayon element which consists in appreciably tensioning the same, and effecting a rearrangement of the filaments toward a parallel relation.
2. The method of lusterizing a spun rayon element which consists in appreciably tensioning the same while in a moist condition, and effecting a rearrangement of the filaments toward a parallel relation.
3. The method of lusterizing a spun rayon element which consists in appreciably tensioning the same while in a moist condition, then drying the tensioned element, and effecting a rearrangement of the filaments toward a parallel relation.
4. The method of lusterizing yarn resulting from cutting rayon filaments into relatively short lengths and, then, spinning the same into a textile element or yarn, which consists in tensioning said element and maintaining it tensioned until substantially dry.

In testimony whereof I affix my signature.  
WOLDEMAR M. STERNBERG.